

# United States Patent

[19]

Ritzen et al.

[11] 3,709,822

[45] Jan. 9, 1973

[54] **METHOD OF MANUFACTURING MAGNET CORES AND MAGNET CORES MANUFACTURED BY THE SAME**

[75] Inventors: **Johannes Maria Jozef Ritzen; Hans Peter Peloschek**, both of Emmasingel, Eindhoven, Netherlands

[73] Assignee: **U.S. Philips Corporation**, New York, N.Y.

[22] Filed: **June 24, 1971**

[21] Appl. No.: **156,573**

[30] **Foreign Application Priority Data**

June 26, 1970 Netherlands ..... 7009421

[52] **U.S. Cl.** ..... **252/62.6, 252/62.61, 252/62.62**

[51] **Int. Cl.** ..... **C04b 35/26**

[58] **Field of Search** ..... **252/62.61, 62.6, 62.62**

[56] **References Cited**

## UNITED STATES PATENTS

2,751,353 6/1956 Gorter ..... 252/62.61

|           |         |                           |             |
|-----------|---------|---------------------------|-------------|
| 2,882,235 | 4/1959  | Gorter et al. ....        | 252/62.61 X |
| 2,986,523 | 5/1961  | Van Der Burgt et al. .... | 252/62.61   |
| 3,033,792 | 5/1962  | Kikuchi.....              | 252/62.61   |
| 3,370,011 | 2/1968  | Kitagawa.....             | 252/62.61   |
| 3,483,126 | 12/1969 | Sara et al. ....          | 252/62.61 X |
| 3,637,504 | 1/1972  | Schmid.....               | 252/62.61   |

## FOREIGN PATENTS OR APPLICATIONS

1,368,160 6/1964 France .....

*Primary Examiner*—James E. Poer

*Assistant Examiner*—J. Cooper

*Attorney*—Frank R. Trifari

[57] **ABSTRACT**

The invention relates to a method of manufacturing magnet cores consisting of representatives of a special class of lithium-, copper-, zinc-, (cobalt-) ferrites, by sintering at temperatures which do not exceed 1100°C. These cores may serve to replace, nickel-containing and hence more expensive, ferrite cores which may serve as "yoke" rings or as aerial rods.

**6 Claims, No Drawings**

**METHOD OF MANUFACTURING MAGNET CORES  
AND MAGNET CORES MANUFACTURED BY THE  
SAME**

The invention relates to a method of manufacturing magnet cores consisting of a soft magnetic ferrite and to ferrite cores manufactured by this method.

Magnet cores which consist of a soft-magnetic ferrite and which on the one hand satisfy three quality requirements to be defined in detail below and which on the other hand are distinguished by comparatively low manufacturing costs formed the object of the examination which has resulted in the present invention.

The said quality requirements are:

- a. the initial permeability  $(\mu_i)$ , measured at a temperature of 23 °C and a frequency of 4 kHz, is higher than 150;
- b. the specific resistivity  $(\rho)$ , measured at a temperature of 23 °C, is higher than 10<sup>6</sup> ohm cm;
- c. the Curie temperature  $(T_c)$ , is higher than 130 °C; the "Curie temperature" is to be understood to mean herein that value of the temperature at which the initial permeability, as a function of the temperature, after having reached its maximum value has fallen with increasing temperature to a value of 10 percent of the said maximum value.

The requirement of comparatively low manufacturing costs implies that the magnet cores in question may not contain nickel and that they can be manufactured by means of a sintering process which requires no temperatures higher than 1100°C and which can be carried out in air.

It was far from easy to manufacture magnet cores in which all the said requirements which mutually are more or less conflicting can be satisfied simultaneously. For example, although magnet cores consisting of manganese-zinc-ferro-ferrite are distinguished by a comparatively high initial permeability, they show a comparatively low specific resistivity, in the order of magnitude of 10<sup>2</sup> ohm.cm, while the sintering temperatures required for the manufacture of said magnet cores are rather high, namely from 1200 °C to 1350 °C. The possibility of realizing soft-magnetic ferrites while using comparatively low sintering temperatures with on the one hand a comparatively high initial permeability and on the other hand a comparatively high resistivity is present, it is true, but one is committed to nickel-zinc-copper ferrites which are comparatively expensive in connection with the nickel present therein. During the preparation of said ferrite, the sintering should often be carried out in an atmosphere which is rich in oxygen.

The invention is particularly suitable for the preparation of so-called "yoke rings" and aerial rods.

"Yoke rings" are to be understood to mean magnet cores consisting of soft-magnetic ferrite and to be used at frequencies varying from 4 to 1000 kHz in deflection coils for television display tubes. Besides the above-mentioned quality requirements b and c, said yoke rings must preferably also satisfy the requirement that the initial permeability should be higher than 300 ( $\mu_i > 300$ ).

Aerial rods to be used at frequencies higher than 1 MHz must satisfy, besides the above-mentioned quality requirements a, b and c, preferably also the following quality requirements:

- d.  $\operatorname{tg} \delta / \mu_i$  (at a temperature of 23 °C and a frequency of 1.5 MHz)  $< 70 \times 10^{-6}$ ;

e. TF (in temperature range from 5 °C to 55 °C, having 23 °C as the reference temperature)  $< 10 \times 10^{-6}$ .

The temperature factor (TF) is the most reliable standard for the temperature dependence of the magnetic initial permeability of the magnet core. It is defined as follows:

$$(TF)_{(t_x-t_r)} = \left( \frac{(\mu_i)_{t_x} - (\mu_i)_{t_r}}{(\mu_i)_{t_r}^2 \cdot (t_x - t_r)} \right)$$

wherein  $(\mu_i)_{t_x}$  is the value of the magnetic initial permeability of the magnet core in question at the temperature  $t_x$ , while  $(\mu_i)_{t_r}$  is the value of the magnetic initial permeability at the reference temperature  $t_r$ . As a rule, and in this case also, room temperature (23 °C) is chosen for the reference temperature  $t_r$ .

The magnet cores manufactured according to the invention consists of soft-magnetic ferrites built up from ferric oxide,  $\text{Fe}_2\text{O}_3$ , copper oxide,  $\text{CuO}$ , lithium oxide  $\text{Li}_2\text{O}$ , zinc oxide,  $\text{ZrO}_2$ , and, possibly, cobalt oxide,  $\text{CoO}$ . These ferrites may be considered as mixed crystal materials having as mixed crystal components cubic ferrite  $\text{CuO} \cdot \text{Fe}_2\text{O}_3$ , zinc ferrite,  $\text{ZnO} \cdot \text{Fe}_2\text{O}_3$ , possibly cobalt ferrite,  $\text{CoO} \cdot \text{Fe}_2\text{O}_3$ , and in addition the ferrite of the bivalent complex  $(\text{Li}_{0.5} + \text{Fe}_{0.5}^{3+})$  which ferrite thus has a composition according to the formula  $(\text{Li}_{0.5} + \text{Fe}_{0.05}^{3B4})\text{O} \cdot \text{Fe}_2\text{O}_3$ . This ferrite is a known material the composition of which in the technical literature is usually referred to by means of the formula  $\text{Li}_2\text{O} \cdot 5 \text{Fe}_2\text{O}_3$  (see, for example, "Naturwissenschaften" 26, p. 431 (1938) and Dutch Pat. specification No. 77,389) which formula is a different notation for the above-mentioned formula:  $(\text{Li}_{0.5} + \text{Fe}_{0.05}^{3+})\text{O} \cdot \text{Fe}_2\text{O}_3$ . The composition of this material in the technical literature is also sometimes referred to by the formula  $\text{Li}_{1/2}\text{Fe}_{2 1/2}\text{O}_4$  (see again the above-mentioned Dutch Pat. specification No. 77,389). A part of the iron oxide of the starting mixture thus takes part in the formation of the bivalent complex oxide  $(\text{Li}_{0.5} + \text{Fe}_{0.5}^{3+})\text{O}$  which, like the other oxides  $\text{CuO}$ ,  $\text{ZnO}$  and possibly  $\text{CoO}$ , forms, with the rest of the iron oxide, a ferrite of the formula  $\text{MeO} \cdot \text{Fe}_2\text{O}_3$  (wherein Me is one of the above-mentioned bivalent metal oxides or the above-mentioned complex metal oxide). It has advantages to state the composition of the starting mixture in molecular percentages of the oxides  $\text{Fe}_2\text{O}_3$  (in as far as this does not contribute to the formation of the complex oxide of the formula  $(\text{Li}_{0.5} + \text{Fe}_{0.5}^{3+})\text{O}$ ,  $\text{CuO}$ ,  $\text{ZnO}$ , possibly  $\text{CoO}$ , and  $(\text{Li}_{0.5} + \text{Fe}_{0.5}^{3+})\text{O}$ , and that for two reasons.

First of all it is found immediately in how far the composition of the starting mixture deviates from the so-called "stoichiometric" composition. "Stoichiometric" composition is to be understood to mean a composition in which the molecular percentage of the iron oxide is equal to the molecular percentage of the oxide  $\text{MeO}$  (with a single ferrite) and is equal to the sum of the molecular percentages of the oxides  $\text{MeO}$  (with a mixed ferrite), respectively, or, in other words, a composition with 50 mol.%  $\text{Fe}_2\text{O}_3$ , not counting iron which would cooperate in the formation of a complex bivalent oxide.

A second advantage of the above-described manner of indicating the composition of the starting mixture is related to the condition that the ratio of the molecular percentages of the complex oxide  $(\text{Li}_{0.5} + \text{Fe}_{0.5}^{3+})\text{O}$  on the one hand and the  $\text{ZnO}$  on the other hand, in the

starting mixtures has been found to be of importance in relation to the magnet cores manufactured from these starting mixtures either or not fulfilling the above-mentioned quality requirements. In other words: the magnetic quality properties of the resulting magnet cores also depend upon the ratio



in the starting mixture.

The method according to the invention is characterized in that a finely divided mixture of iron oxide,  $Fe_2O_3$ , copper oxide,  $CuO$ , lithium oxide  $Li_2O$ , zinc oxide,  $ZnO$ , and, possibly, cobalt oxide,  $CoO$ , having a composition expressed in molecular percentages of the metal oxides, in which the lithium is deemed to be present exclusively as a component of a bivalent complex oxide having a composition according to the formula  $(Li_{0.5} + Fe_{0.5}^{3+})O$ , and in which the iron which would be required for the formation of said complex bivalent oxide is not included in the notation of the quantity of iron, expressed in molecular percentages  $Fe_2O_3$ , which mixture has a composition defined in this manner of:

45.0 – 52.5 mol % of  $Fe_2O_3$ ,

5 – 20 mol % of  $CuO$ ,

0 – 5 mol % of  $CoO$ ,

remainder  $(Li_{0.5} + Fe_{0.5}^{3+})O$  and  $ZnO$ ,

in a ratio varying from 0.25 : 1 to 1.5 : 1, is compressed in the form of the magnet core to be manufacture, after which the resulting compressed product is sintered in air or in a mixture of air and oxygen at a temperature which does not exceed 1100 °C.

As the case may be, the mixture of the above-mentioned metal oxide is prefired at a temperature of at most approximately 950 °C after which the prefired product is cooled, pulverized and compressed in the form of the magnet core to be manufactured, and the resulting compressed product is sintered again in air or in a mixture of air and oxygen at a temperature which does not exceed 1100 °C.

As is known in the preparation of the ferromagnetic ferrites by sintering finely divided mixtures of metal oxides, one or more of the said oxides in the starting mixture may be replaced by another compound of the same metal, which compound can be converted into the corresponding metal oxide during the heating required for the sintering. Such compounds are, for example, carbonates, oxalates and acetates.

For the manufacture of yoke rings according to the invention start is preferably made from mixtures having a composition, defined in the same manner, of

46.5 – 50.5 mol % of  $Fe_2O_3$ ,

5 – 20 mol % of  $CuO$ ,

0 – 2.5 mol %  $CoO$ ,

remainder  $(Li_{0.5} + Fe_{0.5}^{3+})O$  and  $ZnO$ ,

in a ratio varying from 0.25 : 1 to 0.75 : 1.

For the manufacture of aerial rods according to the invention, the starting material preferably are mixtures having a composition, defined in the same manner, of

47.5 – 50 mol % of  $Fe_2O_3$ ,

5 – 15 mol % of  $CuO$ ,

0.7 – 2 mol % of  $CoO$ ,

remainder  $(Li_{0.5} + Fe_{0.5}^{3+})O$  and  $ZnO$ ,

in a ratio varying from 0.25 : 1 to 1 : 1.

By means of the method according to the invention a number of magnet cores were prepared as follows: Starting materials were iron oxide,  $Fe_2O_3$ , copper carbonate  $CuCO_3$ , zinc oxide,  $ZnO$ , lithium carbonate,  $Li_2CO_3$  and, possibly, cobalt carbonate,  $CoCO_3$ . The starting materials were mixed in the desired ratio. The mixture was ground in a ball mill using ethanol as a grinding liquid for 6 hours. The ground product was 5 then filtered off, dried and prefired for one hour by heating it at a temperature of 850 °C. As is known, such a prefiring is a rather universally used measure in manufacturing methods of the type in question. The 10 prefired product was then ground for 16 hours in a ball mill using water as a grinding liquid. The ground product was then filtered off and dried. A binder was added which consisted of 2 percent solution of ammonium alginate in water. The resulting doughy mass 15 was granulated by forcing it through the meshes of a sieve. From the granulate rings were compressed with a pressure of compression of 0.5 ton/cm<sup>2</sup>. The rings were then sintered in air. For that purpose they were heated 20 up to the peak temperature (sintering temperature) at a rate of approximately 150 °C per hour. The rings were maintained at the peak temperature for approximately 15 minutes after which, again at a rate of approximately 150 °C per hour, they were cooled to room 25 temperature.

At least the first three of the following five quality values were measured in each of the resulting annular sintered bodies (magnet cores):

- 35 1. the magnetic initial permeability,  $\mu_i$ , at a frequency of 4 kHz and at a temperature of 23 °C;
2. the Curie temperature,  $T_c$ ;
3. the specific resistivity,  $\rho$ , at a temperature of 23 °C;
- 40 4. the quotient of the loss factor and the initial permeability  $tgp/\mu_i$ , at a temperature of 23 °C and a frequency of 1.5 MHz.
5. the temperature factor,  $TF$ , in the temperature range from 5 °C to 55 °C, with room temperature (23 °C) as a reference point.

The compositions of the starting mixtures, the sintering temperatures ( $T_s$ ) used, and the measured quality values of the resulting magnet cores are recorded in the two following tables, (Tables A and B). In these tables (and also in the subsequent tables C and D) the above-mentioned ratio  $(Li_{0.5} + Fe_{0.5}^{3+})O/ZnO$  is briefly denoted as " $Li_{0.5}/Zn$ ".

55 It is to be noted that it is also possible to heat more quickly, even at a rate of approximately 70 °C per minute. Sintering temperatures lower than stated in the table may also be used subject to the peak temperature being maintained longer, for example, 1 to 2 hours. After the sintering, cooling may also be carried out more quickly, for example, even at a rate of approximately 20 °C per minute. Finally it is stated that the sintering and also the subsequent cooling can also be carried out successfully in an oxygen atmosphere or in a mixture of air and oxygen. However, it is naturally simpler and easier to carry out the sintering in air.

TABLE A

| Magnet core No. | Mol percent   |           |      |       | $T_s$<br>(°C.) | $\mu_i$ | $T_c$<br>(°C.) | $\rho \times 10^{-6}$<br>(ohm. cm.) |
|-----------------|---------------|-----------|------|-------|----------------|---------|----------------|-------------------------------------|
|                 | $Li_{0.5}/Zn$ | $Fe_2O_3$ | CuO  | CoO   |                |         |                |                                     |
| 1               | 0.5           | 50.0      | 5.0  | ----- | 1,096          | 278     | 165            | 4                                   |
| 2               | 0.5           | 50.0      | 10.0 | ----- | 1,056          | 281     | 193            | 12                                  |
| 3               | 0.5           | 50.0      | 15.0 | ----- | 990            | 198     | 225            | 60                                  |
| 4               | 1.0           | 50.0      | 5.0  | ----- | 1,096          | 162     | 293            | 4.7                                 |
| 5               | 1.0           | 50.0      | 15.0 | ----- | 1,040          | 174     | 315            | 2.5                                 |
| 6               | 0.5           | 50.0      | 5.0  | ----- | 1,096          | 278     | 165            | 4                                   |
| 7               | 0.5           | 50.0      | 10.0 | ----- | 1,056          | 281     | 193            | 12                                  |
| 8               | 0.5           | 50.0      | 15.0 | ----- | 990            | 198     | 225            | 60                                  |
| 9               | 0.25          | 50.0      | 15.0 | ----- | 970            | 273     | 145            | 60                                  |
| 10              | 0.5           | 52.5      | 10.0 | ----- | 1,083          | 155     | 230            | 1.9                                 |
| 11              | 0.5           | 51.0      | 10.0 | ----- | 1,083          | 260     | 221            | 2.8                                 |
| 12              | 0.5           | 50.5      | 10.0 | ----- | 1,083          | 318     | 218            | 2.7                                 |
| 13              | 0.5           | 50.0      | 10.0 | ----- | 1,068          | 235     | 210            | 12                                  |
| 14              | 0.5           | 49.5      | 10.0 | ----- | 1,068          | 275     | 205            | 15                                  |
| 15              | 0.5           | 49.0      | 10.0 | ----- | 1,068          | 343     | 230            | 16                                  |
| 16              | 0.5           | 48.5      | 10.0 | ----- | 1,050          | 317     | 192            | 24                                  |
| 17              | 0.5           | 48.0      | 10.0 | ----- | 1,050          | 361     | 185            | 31                                  |
| 18              | 0.5           | 47.5      | 10.0 | ----- | 1,025          | 373     | 180            | 200                                 |
| 19              | 0.5           | 47.0      | 10.0 | ----- | 1,025          | 343     | 173            | 250                                 |
| 20              | 0.5           | 47.0      | 10.0 | ----- | 1,050          | 447     | 173            | 180                                 |
| 21              | 0.5           | 49.0      | 10.0 | 0.5   | 1,060          | 340     | 186            | 22                                  |
| 22              | 0.5           | 49.0      | 10.0 | 1.0   | 1,060          | 320     | 198            | 22                                  |
| 23              | 0.5           | 49.0      | 10.0 | 1.5   | 1,060          | 320     | 197            | 22                                  |
| 24              | 0.5           | 49.0      | 10.0 | 2.5   | 1,060          | 305     | 200            | 20                                  |
| 25              | 0.25          | 50.0      | 10   | 5.0   | 1,090          | 151     | 150            | 8                                   |

TABLE B

| Magnet core No. | Mol percent   |           |      |       | $T_s$<br>(°C.) | $\mu_i$ | $T_c$<br>(°C.) | $\rho \times 10^{-6}$<br>(ohm. cm.) | $tg\delta/\mu_i \times 10^3$ | T.F. $\times 10^3$ |
|-----------------|---------------|-----------|------|-------|----------------|---------|----------------|-------------------------------------|------------------------------|--------------------|
|                 | $Li_{0.5}/Zn$ | $Fe_2O_3$ | CuO  | CoO   |                |         |                |                                     |                              |                    |
| 26              | 0.5           | 49.0      | 10.0 | ----- | 1,040          | 254     | 186            | 7.5                                 | 63                           | 49                 |
| 27              | 0.5           | 49.0      | 10.0 | 0.5   | 1,040          | 238     | 186            | 9                                   | 65                           | 12                 |
| 28              | 0.5           | 49.0      | 10.0 | 1.0   | 1,040          | 226     | 198            | 9                                   | 50                           | 2.0                |
| 29              | 0.5           | 49.0      | 10.0 | 1.5   | 1,040          | 220     | 197            | 8.5                                 | 59                           | 5.0                |
| 30              | 1.0           | 50.0      | 10.0 | ----- | 1,087          | 174     | >150           | 2.5                                 | 140                          | 19                 |
| 31              | 1.0           | 50.0      | 10.0 | 1.0   | 1,087          | 195     | >150           | 2.9                                 | 124                          | 0                  |
| 32              | 1.0           | 49.0      | 10.0 | ----- | 1,061          | 177     | >150           | 16                                  | 80                           | 25                 |
| 33              | 1.0           | 49.0      | 10.0 | 1.0   | 1,061          | 187     | >150           | 25                                  | 61                           | 6.3                |
| 34              | 1.0           | 49.0      | 10.0 | 2.0   | 1,038          | 187     | >150           | 35                                  | 47                           | 9.0                |
| 25              | 1.0           | 48.0      | 10.0 | ----- | 1,038          | 173     | >150           | 200                                 | 62                           | 14                 |
| 36              | 1.0           | 48.0      | 10.0 | 1.0   | 1,038          | 173     | >150           | 500                                 | 37                           | 12                 |
| 37              | 1.0           | 48.0      | 10.0 | 2.0   | 1,038          | 136     | >250           | 500                                 | 40                           | 4.7                |

The following tables C and D relates to magnet cores in the manufacture of which the starting mixture was not prefired but was mixed with the binder after prolonged grinding in a ball mill or a vibratory mill, and processes to a granulate, from which granulate rings were then compressed in the above-described manner, which rings were sintered in air, during which the peak temperature was again maintained for approximately 15 minutes.

TABLE C

| Magnet core No. | Mol percent |           |      |       | $T_s$<br>(°C.) | $\mu_i$ | $T_c$<br>(°C.) | $\rho \times 10^{-6}$<br>(ohm. cm.) | $tg\delta/\mu_i \times 10^3$ | T.F. $\times 10^3$ |
|-----------------|-------------|-----------|------|-------|----------------|---------|----------------|-------------------------------------|------------------------------|--------------------|
|                 | Zn          | $Fe_2O_3$ | CuO  | CoO   |                |         |                |                                     |                              |                    |
| 38              | 0.5         | 51.0      | 10.0 | ----- | 1,083          | 287     | 218            | 7                                   | 7                            | 13                 |
| 39              | 0.5         | 50.5      | 10.0 | ----- | 1,083          | 390     | 208            | 13                                  | 13                           | 16                 |
| 40              | 0.5         | 50.0      | 10.0 | ----- | 1,083          | 420     | 197            | 16                                  | 16                           | 330                |
| 41              | 0.5         | 49.5      | 10.0 | ----- | 1,083          | 530     | 185            | 220                                 | 14                           | 340                |
| 42              | 0.5         | 49.0      | 10.0 | ----- | 1,083          | 560     | 170            | 340                                 | 14                           | 22                 |
| 43              | 0.5         | 48.5      | 10.0 | ----- | 1,083          | 560     | 160            | 340                                 | 14                           | 16                 |
| 44              | 0.5         | 48.0      | 10.0 | ----- | 1,083          | 560     | 149            | 340                                 | 14                           | 16                 |
| 45              | 0.5         | 47.5      | 10.0 | ----- | 1,083          | 640     | 135            | 320                                 | 14                           | 16                 |

TABLE D

| Magnet core No. | Mol percent   |           |     |     | $T_s$<br>(°C.) | $\mu_i$ | $T_c$<br>(°C.) | $\rho \times 10^{-6}$<br>(ohm. cm.) | $tg\delta/\mu_i \times 10^3$ | T.F. $\times 10^3$ |
|-----------------|---------------|-----------|-----|-----|----------------|---------|----------------|-------------------------------------|------------------------------|--------------------|
|                 | $Li_{0.5}/Zn$ | $Fe_2O_3$ | CuO | CoO |                |         |                |                                     |                              |                    |
| 46              | 0.5           | 50.0      | 10  | 0.5 | 1,090          | 390     | 199            | 20                                  | 73                           | 21                 |
| 47              | 0.5           | 50.0      | 10  | 1.0 | 1,090          | 355     | 213            | 20                                  | 65                           | 15.5               |
| 48              | 0.5           | 50.0      | 10  | 1.5 | 1,090          | 295     | 218            | 23                                  | 65                           | 0.8                |
| 49              | 0.5           | 50.0      | 10  | 1.5 | 1,090          | 320     | 228            | 26                                  | 53                           | 5.0                |

What is claimed is:

1. A method of manufacturing a soft-magnetic ferrite core, characterized in that a finely divided starting mixture of iron oxide,  $Fe_2O_3$ , copper oxide, CuO, lithium oxide,  $Li_2O$ , zinc oxide, ZnO, and, cobalt oxide, CoO, having a composition expressed in molecular percentages of the metal oxides of

45.0–52.5 mol % of  $Fe_2O_3$ .

5–20 mol % of CuO,

0–5 mol % of CoO, and the remainder

$(Li_{0.5} + Fe_{0.5}^{3+})O$  and ZnO,

in a ratio varying from 0.25 : 1 to 1.5 : 1, in which the lithium is present exclusively as a component of a bivalent complex oxide of a composition according to the formula  $(Li_{0.5} + Fe_{0.5}^{3+})O$ , and in which the iron which is required for the formation of said bivalent complex oxide is not included in the notation of the quantity of iron, expressed in molecular percentages  $Fe_2O_3$ , is compressed in the form of a magnetic core, and the formed compressed core is sintered in air or a mixture of air and oxygen at a temperature which does not exceed 1100°C.

2. A method as claimed in claim 1, characterized in that the starting mixture has a composition of

46.5–50.5 mol % of  $Fe_2O_3$ ,

5–20 mol % of CuO,

0–2.5 mol % of CuO,

remainder  $(Li_{0.5} + Fe_{0.5}^{3+})O$  and ZnO, in a ratio varying from: 0.25 : 1 to 0.75 : 1.

3. A method as claimed in claim 1, characterized in

4. A method as claimed in claim 1, characterized in that at least one of the metal oxides composing the starting mixture is replaced by a compound of the same metal, which is convertible into the corresponding metal oxide during sintering.

5. A method as claimed in claim 1, characterized in

that the starting mixture is prefired at a temperature of

at most approximately 950°C, cooled, pulverized and

compressed in the form of a magnetic core.

6. A soft-magnetic ferrite core consisting essentially

of a sintered reaction product of

45–52.5 mol % of  $Fe_2O_3$ ,

5–20 mol % of CuO,

0–5 mol % of CoO, and the remainder

$(Li_{0.5} + Fe_{0.5}^{3+})O$  and ZnO in a ratio varying from 0.25:

1 to 1.5 : 1, the iron required for the formation of

$(Li_{0.5} + Fe_{0.5}^{3+})O$  not being included in the the quantity of iron, expressed in molecular percentages as  $Fe_2O_3$ ,

said core having an initial permeability ( $\mu$ ) higher than

150 at a temperature of 23°C and a frequency of 4 kHz,

a specific resistivity ( $\rho$ ) at 23°C higher than  $10^6$  ohm-cm,

and a Curie temperature higher than 130°C.

\* \* \* \* \*

UNITED STATES PATENT OFFICE  
CERTIFICATE OF CORRECTIONPatent No. 3,709,822Dated January 9, 1973Inventor(s) JOHANNES M.J. RITZEN ET AL

It is certified that error appears in the above-identified patent and that said Letters Patent are hereby corrected as shown below:

Column 2, line 13, " $(\mu_i)_t$ " should read  $-(\mu_i)_{tr}-$ ;

Column 2, line 20, "Zr0" should read  $--Zn0--$ ;

Column 2, line 27, change " $Fe_{0.05}^{3BA}$ " to read  $--Fe_{0.5}^{3+}-$ ;

Column 2, line 33, change " $\pm Fe_{0.05}^{3+}$ " to read  $--+ Fe_{0.5}^{3+}-$ ;

Column 2, line 43, change "BD3" to read  $--O_3--$ ;

Column 2, line 60, change "Fe20<sub>3</sub>" to read  $--Fe_2O_3--$ ;

Column 3, line 8, change "Zno" to read  $--ZnO--$

Column 4, line 5, change "Li<sub>2</sub>(O<sub>3</sub>" to read  $--Li_2CO_3--$ ;

Column 4, line 5, change "Co(O<sub>3</sub>" to read  $--CoCO_3--$ ;

Column 5, in TABLE B after "34" in "Magnet core No." column,

change "25" to read  $--35--$ ;

Signed and sealed this 12th day of February 1974.

(SEAL)  
Attest:

EDWARD MFFLETCHER, JR.  
Attesting Officer

C. MARSHALL DANN  
Commissioner of Patents